

# UNITED STATES PATENT OFFICE.

DORWIN D. PENNOYER, OF BOSTON, ASSIGNOR, BY MESNE ASSIGNMENT,  
OF ONE-HALF OF HIS RIGHT TO JESSE S. WILLIAMS, OF LOWELL,  
MASSACHUSETTS.

## COMPOSITION FOR ROOFS.

SPECIFICATION forming part of Letters Patent No. 224,606, dated February 17, 1880.

Application filed October 3, 1879.

*To all whom it may concern:*

Be it known that I, DORWIN D. PENNOYER, of Boston, in the county of Suffolk and State of Massachusetts, have invented an Improved 5 Composition for Roofs and Walls of Buildings, Ships' Bottoms, &c.; and I hereby declare the following to be a full, clear, and exact description thereof.

Heretofore it has been customary to coat 10 roofs with a preparation of coal-tar pitch, and afterward spread over it a layer of gravel to make it water-tight; but this method is objectionable for the reason that when the roof becomes heated by the rays of the sun the pitch 15 blisters or boils and runs, leaving the roof bare in some places and in a leaky condition, and almost impossible to repair and make tight without removing the entire covering.

My invention has for its object to overcome 20 this difficulty; and it consists in a compound formed of certain ingredients combined and treated in such a manner as to produce an elastic covering for roofs, &c., which is capable of successfully resisting the action of heat 25 and water.

I take a suitable vessel and place therein about five gallons of coal-tar and five gallons of raw tar ("raw tar" being the trade designation of Stockholm tar in a raw state) and 30 set it over a fire, and when hot add five pounds of ground rock-salt and ten pounds of flour of lime, and thoroughly incorporate the whole together by stirring. After the mass has become nearly cool I add four pounds of muriatic acid and thoroughly stir the whole together, when it is drawn off into barrels, ready 35 for use.

This compound is applied by means of a brush to roofs and walls of buildings provided 40 with a covering of felt, paper, or other material, after which sand or fine gravel is spread over it, which adheres tenaciously to the compound and forms a cement covering which will effectually exclude water.

45 My improved composition will effectually exclude water when applied directly to the surface of the shingles or boards composing the roof or wall of a building without the ad-

dition of sand or fine gravel, and it may also be applied to ships' bottoms with advantage, 50 as the muriatic acid contained in the compound will prevent barnacles from adhering thereto.

The addition of raw tar to the coal-tar prevents the precipitation of the heavier portions 55 of the latter and the evaporation of its volatile elements.

The ground rock-salt and flour of lime give an elastic body to the compound, while the muriatic acid destroys all the inflammable 60 qualities in the tars, and renders the composition fire-proof.

In ordinary temperatures the composition is sufficiently liquid to allow of its being readily applied, while in cold weather it would 65 be necessary to slightly heat it before using.

My improved compound adheres very tenaciously to any surface to which it is applied; is light, cheap, and durable, and perfectly fire and water proof; retains its elasticity, and 70 will not run or melt by heat. Furthermore, it improves by age and wears smooth.

If the roof should accidentally become broken, it can be easily and cheaply repaired and rendered perfectly tight, which is not the case 75 where roofing compositions as heretofore made are employed.

I am aware that muriatic acid has heretofore been added to paving compounds containing coal-tar or asphaltum; hence I make no broad 80 claim to the addition of said acid to such compounds.

What I claim as my invention, and desire to secure by Letters Patent, is—

The within-described composition for roofs, 85 &c., consisting of coal-tar, raw tar, ground rock-salt, flour of lime, and muriatic acid mixed together in about the proportions named, and used with or without sand or gravel, substantially as and for the purpose set forth. 90

Witness my hand this 29th day of September, A. D. 1879.

DORWIN D. PENNOYER.

In presence of—

W. J. CAMBRIDGE,  
CHAS. E. GRIFFIN.